

## UNITED STATES PATENT OFFICE.

AUGUST E. SCHUTTE, OF NORTHBORO, MASSACHUSETTS.

## ROADWAY CONSTRUCTION.

No Drawing.

Application filed July 29, 1922. Serial No. 578,502.

My invention relates to a method of securing and cementing thin roadway surfaces to their foundations such as Portland cement concrete, brick or other material, and is especially designed to re-surface concrete roadways. The invention resides primarily in a method of rendering the concrete or other surface receptive and retentive of a bituminous coating upon which then can be placed, if desired, a bituminous wearing surface, or the first and original bituminous layer can be used alone.

It is a well known fact that concrete road surfaces after having been in use for a while become scaly and uneven on account of particles or small areas breaking off. Many attempts have been made to renovate such surfaces in various ways and especially by applying bituminous compounds such as tar, asphalt and the like. All these attempts have been unsuccessful. This is primarily due to two factors—one is the moisture inherent in a porous concrete structure, and the other is dust which is always present on a superficial surface of the pavement. If a bituminous material is placed upon such concrete surface, the moisture absolutely prevents adhesion and if the upper surface should be dry, it is always more or less covered with dust which it is impossible to remove, and which prevents the penetration of the bitumen so that upon chilling it scales off and is removed by traffic. If the bituminous material placed upon such a surface is of a thin and oily nature, the dust and the structure itself acts as a filter, permitting the thin oils to penetrate to a short distance, leaving the heavier oils at the surface. In such a case the bituminous layer is only held temporarily for the thin oil penetrates deeper and deeper into the structure, leaving the heavier medium resting on the surface, so that after a short time it scales off exactly as the coatings without thinning fluxing oils.

I have discovered that if a thin layer of asphalt is applied to a concrete road surface at an exceedingly high temperature,—a temperature as high or higher than its flash point—and the asphalt is maintained at such a high temperature in contact with such surface for a short time, two actions take place: First, the asphalt so heated becomes very fluid and penetrating, easily and rapidly entering the pores of the structure. Second, the excessive heat of the penetrat-

ing asphalt evaporates the moisture at the immediate surface of the roadway and it escapes through the thin, limpid asphalt. Since the surface of the asphalt on the concrete structure is very thin, the bubbles formed by the vapor or steam easily burst and allow the steam to escape, while the heat still applied at the surface keeps the asphalt so liquid that it immediately fills the space left by the bursting bubble and forms a continuous thin asphalt surface which is thus keyed to the concrete structure itself and on hardening forms a non-scalable, bituminous surface.

The bituminous surface thus formed is naturally retentive of any bituminous structure subsequently placed upon its top so that it can be thickened to any desired thickness by applying upon it by any suitable means more asphalt composition, or an asphalt composition containing a large percentage of asbestos fibre to toughen it such as is described in my U. S. Letters Patent No. 1,265,259, dated May 7, 1918, or any other suitable tough bituminous layer.

It is a well known fact among engineers and road builders that the wear of a bituminous roadway depends to a great extent upon the bitumen content in the mixture, i. e. the same grade of asphalt being used, a mixture containing a greater amount of such asphalt will be a mixture which will wear longer and better than one having less asphalt, provided the mixture can be kept in place and prevented from shoving and rutting. It has been impossible heretofore to use such rich thin mixtures because no means were found to anchor them to the foundation so that they naturally were shoved and broken up by traffic. If again such rich mixtures were laid thick, while they would resist abrasion, they would not resist the dead weight of traffic and soon formed ruts and channels and became useless.

With my method of anchoring such coatings securely to a rigid concrete foundation, it is possible thereby to cement them to such foundations and so to cover the foundation with a very tough, thin layer of bituminous compound, containing fibres like asbestos, with or without the addition of mineral matter, and thereby produce an excellent roadway. Old concrete roadways can thus be renewed and old bituminous surfaces can be toughened, revived and leveled. Not only is a thin wearing surface applied to the con-

crete by my method, but the concrete itself is toughened and strengthened at the point of contact by being cemented at the line of juncture by two cements, a concrete and bituminous.

5 To practice my invention I proceed as follows:—

Assuming that an old concrete road is to receive the treatment (and for these my 10 method is especially designed): The road is first swept and cleaned to remove all superficial dirt and dust and the tar and filler which is usually found in and about the cracks of the old concrete are removed. The large 15 cracks are then filled by placing in them a bituminous cement and applying superficial heat until the bitumen has entered the pores, crevices and voids on the side of the cracks. The whole surface is then treated 20 by spreading bitumen, either in a liquid form or in the form of powder or chunks, and applying intense heat,—heat which will melt the bitumen and raise it to a temperature above its flash point, such that it may 25 cause the surface being treated to burst into flame, liquefying the asphalt, evaporating the moisture in the concrete and penetrating into it. The distance of penetration depends upon the length of application of the 30 heat, but for paving surfaces the light penetration of a sixteenth of an inch or so is sufficient to secure adhesion, and this can be achieved in a few minutes. The means of heating can be either direct flames, which is 35 the simplest way, or can be superheated steam, superheated air, gas or any other suitable means for producing intense heat. After the surface has thus been treated, it 40 is found that some of the asphalt has penetrated more or less into the structure, leaving the most of it on the surface as a continuous thin layer. Such treatment alone is sufficient for surfaces exposed to pedestrian traffic, such as sidewalks and especially factory 45 floors. For street roadways, however, it is preferable to thicken this bituminous surface. A hot bitumen will stick, adhere to, become commingled with and be retained by a bituminous surface. Therefore to 50 thicken the layer of bitumen on the treated concrete surface, it is only necessary to apply a secondary coating of a rich bituminous mixture at a temperature hot enough to melt or soften the bitumen below, so that 55 the two layers will coalesce. This secondary

coat, if such is used, is preferably one composed of asphalt, having incorporated therewith short asbestos fibre and, if desired, some sand, and applied at a heat of about 60 350 degrees Fahrenheit; or a rich mixture of sand and bitumen can be applied or, in fact, any rich, tough, bituminous composition. These can be troweled on or placed there by any suitable machine and after 65 being slightly chilled, are treated with a superficial scattering of clean sand, which will not penetrate the structure itself, but will lie on the top and be slowly impressed into the surface by traffic, giving the structure a gritty, sand-paper-like surface.

70 While my invention relates especially to the repair of concrete surfaces, it may be used with such surfaces when freshly laid, or in fact with any surfaces to which it is necessary to bind a bituminous layer. In 75 using the term "roadway" I mean to include any wearing surface subject to travel of any kind such as highways, sidewalks, floors, etc., and in using the term "foundation" I mean the surface which receives the 80 bituminous coating and to which such coating is to be united, whether it be made of concrete, bitumen or other material, for the essence of my invention relates to the maintaining of the coating at a temperature approximately or above its flash point, whereby 85 its temperature will effect a penetration of the foundation by the coating or the intermingling of the two so that they are tied together.

90 What I claim as my invention is:—

1. That method of uniting a bituminous coating to a concrete roadway surface which consists in applying said coating to said surface and raising it to a temperature approximating its flash point and maintaining it at such temperature for a short period of time whereby a portion of it will penetrate 95 said surface and the remainder will form a protective coating therefor.

100 2. A method of adding a bituminous layer to a concrete surface which consists in heating the concrete, applying a bituminous compound such as asphalt, heating said asphalt to its flash point whereby it will enter the pores and evaporate the moisture, and then applying a secondary wearing surface thereto.

AUGUST E. SCHUTTE.